# EUROPEAN PATENT SPECIFICATION

(11) **EP 0 308 759 B1**
(45) Date of publication and mention of the grant of the patent: **09.12.1992**
(21) Application number: 88114875.3
(22) Date of filing: 12.09.1988
(51) Int. Cl.: C22C 9/08, C10M 111/00

(54) **Shockproof, wearproof metal lubricant, with restoring action and relative manufacturing process**
Schlagbeständiger und abnutzungsbeständiger metallischer Schmierwerkstoff mit restaurierender Wirkung und diesbezügliches Herstellungsverfahren
Lubrifiant métallique résistant aux chocs et à l'usure présentant un effet de rénovation, ainsi que procédé de fabrication de ce produit

(30) Priority: 24.09.1987 IT 2201687
(43) Date of publication of application: 29.03.1989
(73) Proprietor: LUBRALLOY S.R.L., I-20133 Milano (IT)
(72) Inventor: Trotta, Nicola, Milano (IT)
(74) Representative: Lecce, Giovanni

(56) References cited:
- GB-A- 488 590
- GB-A- 699 097
- GB-A- 785 936
- GB-A- 823 357

## Description

This invention refers to a shockproof, wearproof metal lubricant with restoring action of worn metal surfaces and the relative production process.

As noted, the task of lubrication is to increase the mechanical efficiency of the machines, through a reduction of the friction between moving surfaces rubbing against each other, and to prevent or reduce wear on said moving parts, increasing their lifespan, by placing between them a veil of greasy substances more or less viscous than the lubricants, and help to maintain a suitable thermic state, subtracting continuous heat from the machine.

Although the lubricating action may be exercised by both solid and liquid, gaseous lubricants, in practice liquid or semisolid lubricants, like oil or lubricating grease, are almost exclusively used. The solid lubricants comprise graphite, talc, bentanite and molybdenum bisulphide, all substances with a lamellar structure, almost always used in suspension of liquids, e.g. graphitic oils. Also noted is the use of metal powders which act as support to the liquid or semisolid lubricants to improve their poor shockproof and wearproof qualities. The interest in attempting to use metal products is based on the necessity to form a permanent protective layer on the mechanical moving parts submitted to friction. The metal powders, added to traditional lubricants, serve, in fact, to fill the natural pores and flaws, invisible to the naked eye, of the metal surfaces of the moving mechanical parts subject to wear. The results obtained with the use of metal powders are a reduction of friction, an increase in flowability, a lowering of the operating temperature and rate of wear, an improvement in lubrication, a restoration of the clearances and coupling provided by the constructor and consequently a reduction also in energy consumptions. Among the most tested metals appears, in first place, lead, which offers excellent lubricating and anti-seizing qualities. However, due to its too low melting point (327.5°C), it has never been possible to use this metal as auxiliary for traditional lubricants.

To solve this problem, it has been proposed to encapsulate the lead in another metal with a higher metling point and at the same time flexible; the metal used for this purpose is copper, which has a melting point of 1083°C.

This solution, while making it possible to obtain products with satisfactory characteristics, does not solve the problems linked with the various types of friction, wear and lubrication of the different mechanical systems for which these products are to be used, due to the unstable structure of said products, problems of approximate micronization, oleosolubility and excessive operating cost.

The object of this invention is to optimize the copper and lead alloy so that it may be used for the formulation of lubricating products free from the above problems.

Another object of this invention is to provide a copper and lead alloy which can be dispersed in traditional liquid or semisolid lubricants and solves all problems linked with different types of friction, wear and lubrication of the various mechanical systems.

According to a general aspect of this invention, these objects are obtained by adding to the copper-lead alloy other metals with function of activators.

The object of this invention is therefore a shockproof, wearproof lubricant with restoring action of the worn metal surfaces, consisting of a stable, homogeneous dispersion of microspheres of a quaternary alloy of copper, lead, tin and silver in a mixture of naphthene and paraffin oils.

The microspheres of the alloy can be obtained by means of melting and subsequent process of atomization in a micronized spheric powder in various measures. Its spheric structure, with respect to the lamellar one, offers the advantage of a greater flowability on the surface to be treated, and, in the case of unsuitable thicknesses, ejection or non-reception. The new formulates, specific for lubricants for the lines Industry, Car Drive in general and Navigation, are also characterized by the fact of comprising also special auxiliary substances which must stabilize, standardize and often all keep in suspension, in the mixture of paraffin and naphthene oils, the microspheres of quaternary alloy to guarantee complete homogeneity and stability of said formulates.

The alloy used in the manufacture of the lubricants of this invention can be obtained by means of melting and subsequent atomization process of the metals in the following preferred quantities:
COPPER, between 40 and 60%, preferably 56%, with respect to the weight of the alloy;
LEAD, between 30 and 50%, preferably 40%, with respect to the weight of the alloy;
TIN, between 1 and 5%, preferably 3%, with respect to the weight of the alloy;
SILVER, between 0.1 and 2%, preferably 1%, with respect to the weight of the alloy.

The quaternary alloy is present in the various types of lubricants in quantities of between 12 and 16% in weight and preferably 14% in weight of the total lubricant composition. The most important metal to be put in oily suspension, and, using the lubricant, distributed in all points affected by said lubrication, is lead, as it is well known that it has a high lubricating power.

Due to its low melting point (327.5°C), however, it must be encapsulated, as already mentioned, in another metal, copper, with characteristics of considerable flexibility, but a higher melting point (1083°C). The copper, encapsulated in the quaternary alloy dispersed in the oily phase, does not cause phenomena of oil oxidation as said phenomena are prevented by the antixodiating agents present in the formulates. Tests made by the applicant have shown that this stabilizing action of said antioxidating agents is improved by the addition, during melting of the alloy, of small quantities of silver.

These tests have also demonstrated that the presence of tin seems to improve the anchoring of the microspheres of said alloy to the surfaces to be treated. It is also noted that, in general, tin exercises stabilizing properties in shockproof alloys.

Through atomization of the alloy different fractions of various grain sizes are separated, usable according to the sections to which the various formulates are destined. In fact, if a grain size too fine for the needs of the parts to be treated is used, more time is necessary to obtain satisfactory results, while, if too coarse a grain size is used, it is probable that it does not find a sufficient entrance angle among the surfaces to be treated. This, while not causing problems for the treated parts, does not permit results sufficiently appreciable to justify their use to be obtained. The microspheres are therefore separated in various fractions, generally four, with different diameter intervals, usable for the formulation of four main types of metal lubricants in the following sectors:

| Diameter in microns | Sector | Use/Destination |
|---|---|---|
| 0.1 to 40 | Car drive (and motor cycling) | 2 and 4-stroke diesel and petrol engines |
| 40 to 60 | Car drive | Transmissions, gear-shifts, differential gears); |
| | Industry | compressors, pumps, small reduction gears; |
| | Navigation | transmissions, gear-shifts, U-drive,V-drive etc.; |
| 60 to 90 | Industry | Pinions for lamination trains, pumps, hoisting reduction gears, convertors, cog-wheels, helical gears, etc.; |
| 90 to 115 | Industry | Any type of industrial plant where excessive clearances and wear are found, e.g. in old and neglected plants. |

The above does not, however, limit the field of application of said alloy as it has been experimentally demonstrated that it is possible to use fractions with different grain size interval from that comprised between 0.1 and 115 microns; for example, grain sizes over 115 microns to prepare formulates for specific uses and destinations and particulars different from those indicated.

The composition of the four main formulates prepared with the four grain size fractions of quaternary alloy previously indicated is shown in table A, where the raw materials and relative percentages, the characteristics and function of each of them are specified.

The products obtained are compatible and perfectly mixable with any lubricating oil for either engines or transmissions, but are not compatible with oils additivated with graphite or molybdenum bisulphide and with other solid lubricants. They are suitable for each type of lubrication of any metal surface, both sliding and rolling, with circulation of the lubrication or with fixed chamber. For example, for rapid engines with internal combustion, tests carried out by the applicant have established that, in any type of lubrication, a quantity of metal lubricant not exceeding 4% in weight is recommended.

Greater quantities do not, however, create problems for the treated parts, but represent a useless excess cost. The job of the metal microspheres dispersed in the oily matrix is to reach, transported by normal lubricant, all lubricated points of the parts to be treated, deposit themselves at the scorings, abrasions or pittings, and, exploiting the mechanical action of said part and the heat produced by friction, weld together until they restore optimal conditions of the piece.

This protective film protects, through time, the actual piece, withstanding its loads and future wear and improving, according to the shockproof properties of the mixture, its operation.

The improvements obtainable with said metal lubricant on mechanical parts in general are:
- notable reduction of friction;
- high, constant reduction of energy conumptions, restoring them to the minimum values provided by the constructor;
- reduction of noise by many decimals;
- reduction of approximately 20°C in the operating temperature of the parts treated;
- possibility of planning and reducing maintenance costs, with consequent decrease of machine stops and rise in productivity.

In endothermic petrol engines, the following improvements can also be obtained:
- restoration of compression;
- reduction of lubricant and fuel consumptions;
- wear locking in its state at the moment of the first application, by means of continuous intervention;
- restoration of the tolerance and clearances provided by the constructor.

The diameter interval within which said metal lubricant can be used without undergoing substantial modifications of quality and characteristics is very wide and varies from -200° to +800°C.

The properties of the metal microspheres of being naturally self-lubricating makes it possible to create, within the diameter limits indicated, a self-lubrication process of the treated parts, even when faults or temporary breaks in lubrication take place, with consequent overheating of said parts, guaranteeing, when temperatures do not exceed 830°, the prevention of seizing.

Table B shows the results of some technical tests to which the metal lubricant produced and only the quaternary alloy were submitted. Said tests were carried out with the 4-sphere SHELL EP machine at the Testing Station for the Oil and Grease Industries of Milan, operating on samples of lubricating oil in its present state additivated with the metal lubricant produced with 60 micron alloy (lubricating 60 micron alloy (lubricating oil/metal lubricant ratio = 97/3) and on samples of lithium and silicone grease in their present state additivated with quaternary alloy in powder from 63 to 115 micron (ratio of grease/alloy in powder = 70/30). These results emphasize the highly positive effects obtained in presence of both the metal lubricant and only the alloy in powder as regards the seizing and welding loads and the rate of load/wear and demonstrate the excellent shockproof and wearproof properties also of only the quaternary alloy which forms the base of the metal lubricant.

### Manufacturing process of the lubricant of this invention

In a preparation tank, equipped with stirrer and Cowless movable dispersor turbo, are mixed, at environmental temperature and in equal parts, pure naphthene oil with a viscosity of 26 Cp at 40°C (2.7 Engler at 50°C) and pure paraffin oil with a viscosity of 86 cP at 40°C (8 Engler at 50°C). Said oils will be present, according to the type of lubricant formulated, in a percentage in weight comprised between 68% and 74% of the total. The mixture thus obtained is stirred at 1200 r.p.m. with 40 disk strokes per minute, said stirring representing the optimal value to guarantee total dispersion of the components subsequently inserted. At this point the addition of the other raw materials starts, each taken in the proportions indicated in table A.

First the colloidal mixture with suspending action formed by the metal lithium and dodecylhydroxystearic acid components is inserted, continuing stirring for the time necessary for its complete dispersion, at any rate until, with a dripping test, there are no lumps or deposits of said mixture. Said dripping test will then be repeated after the insertion of each other component. The following are then loaded in this order, the thixotropic agent uncompressed silica gel, the greasy, absorbent agent trioleate glyceryl, the mixture with wearproof, rustproof, detergent action, formed by components metal zinc, metal magnesium and phosphor and the alloy in copper, lead, tin and silver powder (56%-40%-3%-1%). After obtaining perfect distribution and homogeneity of the product and at any rate always and only as last component, is inserted, to improve viscosity and lower freezing point, the linear copolymer of olefins (ethylene-propylene copolymer). Stirring continues to disperse everything well for several minutes, then interrupted and the product allowed to rest for not less than 12 hours, time necessary to determine the thixotropicity necessary to guarantee an effective, constant suspending action of the alloy in powder.

During this period, the preparation tank must not be submitted to agitation or vibrations of any type (ultrasounds included), to avoid damaging the product.

The above process is started, as mentioned, at environmental temperature, but the friction produced by the COWLESS dispersor causes, through time, an inevitable rise in the temperature of the mixtures, which must be kept within 50-55°C to avoid creating problems to the end product.

To maintain temperature within the above limits, the tank is contained in thermostat bath.

## Claims

1. Metal shockproof, wearproof lubricant, with restoring action of worn metal surfaces, consisting in a stable, homogeneous dispersion of microspheres of a quaternary alloy of copper, lead, tin and silver in a mixture of naphthene and paraffin oils.

2. Metal lubricant according to claim 1 , characterized by the fact that said quaternary alloy comprises:
40-60% in weight of copper, preferably 56%; 30-50% in weight of lead, preferably 40%; 1-5% in weight of tin, preferably 3%; and 0.1-2% in weight of silver, preferably 1%.

3. Metal lubricant according to claim 1 or 2, characterized by the fact that the microspheres of said metal alloy have a diameter comprised between 0.1 and 115 microns.

4. Metal lubricant according to any of the previous claims, characterized by the fact that said quaternary alloy is present in quantities comprised between 12% and 16%, preferably 14% in weight of the lubricant.

5. Metal lubricant according to any of the previous claims, characterized by the fact that the mixture of mineral oils is composed 50% of napthene oil with a viscosity of 26 cP at 40°C (2.7 Engler at 50°C) and 50% of paraffin oil with a viscosity of 86 cP at 40°C (8 Engler at 50°C).

6. Metal lubricant according to any of the previous claims, characterized by the fact that the mixture of mineral oils is present in quantity comprised between 68 and 74% in weight, with respect to the lubricant.

7. Metal lubricant according to any of the previous claims, characterized by the fact that it also comprises:
- 1.1 to 2% in weight, with respect to the lubricant, of a colloidal mixture with suspensive action;
- 5 to 7% in weight, with respect to the lubricant, of a thixotropic agent;
- 2.14 to 5.24% in weight, with respect to the lubricant, of an agent with greasy, absorbent action;
- 0.76% in weight, with respect to the lubricant, of additives with wearproof, detergent and rustproof action, and
- 3% in weight, with respect to the lubricant, of an agent which improves viscosity and lowers the freezing point.

8. Metal lubricant according to any of the previous claims, characterized by the fact that it is added in quantity not exceeding 4% by weight of the lubricating oils for both engines and transmissions.

## Patentansprüche

1. Stoss- und verschleissfestes Metall-Schmiermittel, das abgenutzte Oberflaechen wieder instandsetzt, bestehend aus einer stabilen, homogenen Dispersion von Mikrokuegelchen einer Quarternaerlegierung aus Kupfer, Blei, Zinn und Silber in einer Mischung aus Naphten- und Paraffinoelen.

2. Metall-Schmiermittel gemaess Anspruch 1, dadurch gekennzeichnet, dass die besagte Quaternaerlegierung folgendes enthaelt:
40-60% in Gewicht an Kupfer, vorzugsweise 56%: 30-50% in Gewicht an Blei, vorzugsweise 40%; 1-5% in Gewicht an Zinn, vorzugsweise 3%; und 1-2% in Gewicht an Silber, vorzugsweise 1%.

3. Metall-Schmiermittel gemaess Anspruch 1 oder 2, dadurch gekennzeichnet, dass die Mikrokuegelchen besagter Metall-Legierung einen Durchmesser aufweisen, der zwischen 0,1 und 115 Mikron liegt.

4. Metall-Schmiermittel gemaess einem beliebigen der o.g. Ansprueche, dadurch gekennzeichnet, dass besagte Quaternaerlegierung in Mengen vorhanden ist, die zwischen 12% und 26% liegen, und zwar vorzugsweise 14% in Gewicht des Schmiermittels betragen.

5. Metall-Schmiermittel gemaess einem beliebigen der o.g. Ansprueche, dadurch gekennzeichnet, dass die Mischung der Mineraloele zu 50% aus Naphtenoel mit einer Viskositaet von 26 cP bei 40° (2,7 Engler bei 50°C) und zu 50% aus Paraffinoel mit einer Viskositaet von 86 cP bei 40°C (8 Engler 6 bei 50°C) besteht.

6. Metall-Schmiermittel gemaess einem beliebigen der o.g. Ansprueche, dadurch gekennzeichnet, dass die Mischung der Mineraloele in einer Menge vorhanden ist, die zwischen 68 und 74% in Gewicht im Verhaeltnis zum Schmiermittel liegt.

7. Metall-Schmiertmittel gemaess einem beliebigen der o.g. Ansprueche, dadurch gekennzeichnet, dass es ebenso folgendes enthaelt:
- 1,1 bis 2% in Gewicht, im Verhaeltnis zum Schmiermittel, einer Kolloidalmischung mit Suspensivwirkung
- 5 bis 7% in Gewicht, im Verhaeltnis zum Schmiermittel, eines thixotropen Wirkstoffs
- 2,14 bie 5,24% in Gewicht, im Verhaeltnis zum Schmiermittel, eines Wirkstoffs mit fettiger, absorbierender Wirkung;
0.76% in Gewicht, im Verhaeltnis zum Schmiermittel, eines Zusatzes mit verschleissfester, reinigender und rostbestaendiger Wirkung, und
- 3% in Gewicht eines Wirkstoffs, im Verhaeltnis zum Schmiermittel, der die Viskositaet verbessert und den Gefrierpunkt senkt.

8. Metall-Schmiermittel, gemaess einem beliebigen der o.g. Ansprueche, dadurch gekennzeichnet, dass es in einer Menge beigegeben wird, die 4% an Gewicht der Schmieroele fuer beide, sowohl Motor wie Uebersetzungen, nicht ueberschreitet.

## Revendications

1. Métal resistant aux chocs, lubrifiant contre l'usure, avec une action de restauration des surfaces du métal usé, consistant en une dispersion stable et homogène de microsphères d'un alliage quaternaire de cuivre, plomb, étain et argent dans un mélange de naphthène et huile de paraffine.

2. Métal lubrifiant selon la revendication 1, caractérisé par le fait que le dit quaternaire alliage comprend:
40-60% en poids de cuivre, de préférance 56%; 30-50% en poids de plombe, de préférence 40%; 1-5% en poids d'étain, de préférance 3%; et 0,1-2% en poids d'argent, de préférance 1%.

3. Métal lubrifiant selon les revendications 1 et 2, caractérisé par le fait que les microsphères du dit alliage métallique ont un diamètre compris entre 0,1 e 115 microns.

4. Métal lubrifiant selon n'importe quelle précédente revendication, caracterisé par le fait que le dit quaternaire alliage est présent en quantités comprises entre 12% et 16%, de préférence 14% en poids du lubrifiant.

5. Métal lubrifiant selon n'importe quelle revendication précédente, caracterisé par le fait que le mélange des huiles mineraux est composé de 50% de naphthène avec une viscosité de 26 cP à 40°C (2,7 Engler à 50°C) et 50% d'huile de paraffine avec une viscosité de 86 cP à 40°C (8 Engler à 50°C).

6. Métal lubrifiant selon n'importe quelle revendication précédente, caracterisé par le fait que le mélange des huiles mineraux est présent en quantités comprise entre 68% et 74% en poids, par rapport au lubrifiant.

7. Métal lubrifiant selon n'importe quelle revendication précédente, caracterisé par le fait qu'il contient aussi:
- de 1,1 jusqu'à 2% en poids, par rapport au lubrifiant, d'un mélange colloïdal avec une action de suspension;
- de 5 jusqu'à 7% en poids, par rapport au lubrifiant, d'un agent tixothrope;
- de 2,14 jusqu'à 5,24% en poids, par rapport au lubrifiant, d'un agent avec une action absorbante du gras.
- 0,76% en poids, par rapport au lubrifiant, d'additifs avec une action détèrgente et de protection contre l'usure et contre la rouille, et
- 3% en poids, par rapport au lubrifiant, d'un agent qui améliore la viscosité et abaisse le point de congélation.

8. Métal lubrifiant selon n'importe quelle revendication précédente, caracterisé par le fait que sont ajoutés en quantité pas excédente le 4% en poids des huiles lubrifiants pour moteurs et transmissions.
